

Patented Aug. 31, 1926.

1,597,880

# UNITED STATES PATENT OFFICE.

WILLIAM D. GREGOR, WESLEY M. OSBORNE, AND ALEX J. KEMZURA, OF NEWTON FALLS, NEW YORK.

## BLEACHING PROCESS.

No Drawing.

Application filed July 14, 1924. Serial No. 725,982.

The present invention relates to a process for bleaching materials.

More particularly the invention relates to a process for bleaching cellulosic materials, such as pulp used in the manufacture of paper, papier-mâché and like products.

In the usual bleaching processes, such as are commonly used for the preparation of pulp in the manufacture of high grade white papers, to attain the desired degree of whiteness in the stock, it is necessary to sacrifice the strength, hydrating, beating, and other desirable qualities thereof. The difficulty of bleaching fibre produced from hard woods is well known and the bleaching of hard wood fibre made by the sulphite process has heretofore been commercially impracticable.

The objects of the present invention are to provide a process for bleaching materials in which the amount of bleach necessary and the bleaching time are substantially reduced; to provide a bleaching process in which a higher degree of whiteness and improved strength and other desirable qualities may be attained in the stock than has heretofore been obtainable; to provide a commercially practical process for pulps which have not been heretofore practically bleachable; and such other objects as may be attained by utilization of the various steps hereinafter set forth and claimed.

In the usual bleaching processes, the bleach solution is added to the pulp to be bleached, and the mass is heated to speed the reaction. The pulp remains in the bleaching vats until the desired degree of bleach has been reached. In these processes of bleaching, the various desirable qualities, such as strength, beating, and hydration qualities are materially injured.

By dividing the bleaching operation into two stages and treating in accordance with the present invention, it is possible to effect a material saving in bleaching time and in the amount of bleach used, and a superior fibre is produced. In carrying out the invention, the unbleached pulp, as it comes from the stock pits, and having been washed, screened and thickened in the usual way, is pumped or flowed into the bleachers. As the pulp enters the bleachery a small amount of unheated bleaching agent is continuously added to and uniformly mixed with the pulp. The amount of bleach added in this stage

varies with the bleaching quality of the pulp and is preferably about twenty-five to thirty per cent of the total amount required to produce a standard white color in the stock being treated. In practice this amount varies from three to six per cent bleach, based on thirty-five per cent bleach powder. The bleach immediately becomes active as it is thoroughly mixed with the pulp during the filling, avoiding necessity for initial heating. The bleaching agent is allowed to soak thoroughly into the stock until exhaustion of the bleach is reached. As exhaustion is approached the temperature of the mixture is raised to speed the reactions. The time ordinarily required for the bleaching agent to reach exhaustion is from ten to fifteen minutes. As no heat is applied until exhaustion of the agent is approached, no appreciable burning, weakening, or deterioration of the quality of the fiber occurs in this stage. The reactions in this stage proceed until the bleaching agent is exhausted, which condition is indicated by the color of the stock. Usually when the pulp is first contacted with the bleach, the mass assumes a darkened color, and gradually bleaches to a light yellow or cream cast which may be taken as an indication that the end of the first stage has been reached. The color varies with the character of material from which the pulp is produced, the pulps from hard wood being much darker than soft wood pulps, but each kind of pulp has a characteristic color ranging between 50 and 60 in the standard color scale by which the exhaustion of the bleaching agent may be recognized.

The standard color scale herein referred to is the scale adopted by the Technical Association of the Pulp and Paper Industries, and the readings are determined by the aid of a standard tint photometer or by the use of the standard color wheel adopted by the Technical Association. The standard tint photometers measure the percentage of red, green and blue in the pulp, and as the blue governs the white, the per cent of blue is taken as the color of the pulp. The readings are determined in accordance with the scales supplied with the standard instruments. A full disclosure of the standard color scale, herein referred to, and its method of application is given on pages 66

and 67 of the papers of the Technical Association of Pulp and Paper Industries, published June, 1924.

It will also be understood that the quantity of bleach to be added in this stage will vary with the bleaching quality of the stock, and the most effective amount for each kind of stock should be determined by trial.

When the point of exhaustion of the bleaching agent is reached, the stock is removed from the bleachery and thoroughly washed to remove the exhausted agent, the products of the reactions, and other foreign substances which may now be removed by the washing operation. The washed stock is then at the end of the first saving stage, in partially bleached condition, and with the fibers substantially uninjured.

The washed half bleached material is then subjected to the second stage of the treatment which comprises treatment with a new solution of bleach sufficient in quantity to produce the desired degree of whiteness, preferably a standard white color. This may be carried out as in the first stage by adding unheated bleach of proper strength continuously and uniformly to the half bleached stock as it is flowed into the vats, and as the bleaching agent becomes exhausted, the temperature of the mixture may be raised, or the entire second stage may be carried out at a slightly higher temperature. In practice the initial temperature of the first stage is ordinary water temperature, and towards the end of the reaction in the first stage a temperature of 70 degrees F. with a temperature of 85 degrees F. in the second stage, has given excellent results. Ordinary bleach processes are carried out at about 100 degrees F. After the standard white color is attained, the stock is again washed and the bleaching operation is complete.

In actual operation of the invention it has been found that a material improvement is effected when any of the known bleaching agents are used, such for example, as the various liquids, gases or powdered forms, and bleach in any form may be used. It has been further found that after the dilute bleach has been added, if such agents as sulphurous acid or sodium bi-sulphite are added, chlorine is liberated which is taken up in the stock. The addition of such agents are preferred in the first stage as the reaction takes place in a short time and the chlorine is liberated in slight bleaching amounts, effecting an improvement in operation.

By actual test in the use of the present process as compared with regular bleaching methods, a saving of twenty to thirty percent in bleaching time and a material saving in amount of bleach has been effected, while the strength, hydrating and beating

qualities of the pulp are greatly improved, and the pulp is generally superior to that produced by regular methods. The results obtained in the saving of bleach when treating pulps from the same cook are shown in the following tabulation:

| Regular method, bleach used. | Character of pulp. | Improved double bleach process, bleach used. | Saving.   |
|------------------------------|--------------------|----------------------------------------------|-----------|
| Per cent.                    |                    | Per cent.                                    | Per cent. |
| 16.6                         | Spruce.            | 11.5                                         | 4.1       |
| 22.1                         | Hemlock.           | 14.0                                         | 8.1       |
| 15.2                         | Poplar.            | 10.1                                         | 5.0       |
| 30.4                         | Hardwood.          | 16.4                                         | 14.0      |

75

80

It will be noted that by use of the present invention a remarkable saving in bleach is effected in addition to the improvement in the quality of the bleached product noted.

In addition to being stronger, the fiber produced by the present invention is more opaque, and the effect of the slight bleaching action on the fiber walls in the first stage prevents any substantial deteriorating effect in the second stage, even though a stronger solution is used in the second stage. It will be noted that for hardwoods the maximum bleach in the first stage is about 5 or 6%, leaving about 10.5 or 11% in the second stage, whereas in the regular method, the pulp is subjected to 30.4% bleach. The wide difference in strength of the bleach applied to the fiber and the lower temperatures used results in the increased quality in the bleached product produced by the present invention.

So far as known, no prior commercial process for bleaching fibre produced from hardwood by the sulphite process has been successful. By treatment in accordance with the present invention hardwood sulphite pulp may be successfully bleached to a standard white and the product is a high grade fiber.

Having described a preferred embodiment of the invention, what is desired to be secured by Letters Patent and claimed as new, is:

1. In the process of bleaching cellulosic material, the steps which comprise partially bleaching the same, and then intimately contacting the partially bleached material with a bleaching agent in an amount sufficient to bleach the said material to the desired degree at a temperature of approximately 85° F. 115

2. In the process of bleaching cellulosic material, the steps which comprise partially bleaching the same, washing the treated material, and then intimately contacting the partially bleached material with a bleaching agent in an amount sufficient to bleach the said material to the desired degree at a temperature of approximately 85° F. 125

130

3. The process of bleaching paper pulp which comprises intimately commingling the pulp in a wet and unbleached state with a bleaching agent in an amount sufficient only 5 to partially bleach same at a temperature of about 70° F., and intimately contacting the partially bleached pulp with a bleaching agent in an amount sufficient to bleach the pulp to the desired degree at a temperature 10 of approximately 85° F.

4. The process of bleaching paper pulp which comprises intimately commingling the pulp in a wet and unbleached state with a bleaching agent in an amount sufficient only 15 to partially bleach same at a temperature of about 70° F., washing the partially bleached pulp, and intimately contacting the partially bleached pulp with a bleaching agent in an amount sufficient to bleach the pulp to the 20 desired degree at a temperature of approximately 85° F.

5. The process of bleaching paper pulp which comprises intimately commingling the pulp in a wet and unbleached state with a bleaching agent in an amount sufficient only 25 to partially bleach same at a temperature of about 70° F., permitting the reaction to proceed until the activity of the bleaching agent is substantially exhausted, washing the partially bleached pulp, and intimately contacting the partially bleached pulp with a bleaching agent in an amount sufficient to bleach the pulp to the desired degree at a temperature of approximately 85° F.

In testimony whereof, I affix my signature.  
W. D. GREGOR.

In testimony whereof, I affix my signature.  
W. M. OSBORNE.

In testimony whereof, I affix my signature.  
ALEX J. KEMZURA.